

1,089,561.

L. E. HOWARD.  
METHOD OF MAKING INGOTS.  
APPLICATION FILED MAY 7, 1913.

Patented Mar. 10, 1914.

3 SHEETS—SHEET 1.



Witnesses.

*S. J. Mann.*

S. N. Pond

S. N. Pond By Offield, Dowle, Grav. Offield.

संस्कृतः

L. E. HOWARD.  
METHOD OF MAKING INGOTS.  
APPLICATION FILED MAY 7, 1913.

1,089,561.

Patented Mar. 10, 1914.

3 SHEETS-SHEET 2.



Witnesses,

S. D. Mann

D. H. Pond

Inventor,  
Leslie E. Howard,  
By Offield, Taile, Graven Offield

L. E. HOWARD.  
METHOD OF MAKING INGOTS.  
APPLICATION FILED MAY 7, 1913

1,089,561.

Patented Mar. 10, 1914.

3 SHEETS—SHEET 3.



Wittewer,

Dr. D. Mann.

S. N. Pond

By Offield, Towle, Graven-Offield,  
Am's.

*Ames*

# UNITED STATES PATENT OFFICE.

LESLIE E. HOWARD, OF LOCKPORT, NEW YORK, ASSIGNOR TO SIMONDS MANUFACTURING COMPANY, OF FITCHBURG, MASSACHUSETTS, A CORPORATION OF MASSACHUSETTS.

## METHOD OF MAKING INGOTS.

1,089,561.

Specification of Letters Patent. Patented Mar. 10, 1914.

Application filed May 7, 1913. Serial No. 766,095.

*To all whom it may concern:*

Be it known that I, LESLIE E. HOWARD, a citizen of the United States, residing at Lockport, in the county of Niagara and 5 State of New York, have invented certain new and useful Improvements in Methods of Making Ingots.

This invention relates to the art of manufacturing metal ingots, being designed 10 chiefly for use in the manufacture of steel ingots.

In my Letters Patent No. 1,056,101, dated March 18, 1913, I have disclosed an ingot casting and compression machine wherein 15 a two-part, separable ingot mold is located directly above and in vertical alinement with the compression die to receive the molten charge poured therein, and means are provided for opening the mold after the ingot has reached the state of partial solidification and lowering the partially cooled ingot therefrom directly into an underlying compression die. In a companion application filed May 3, 1913, Serial No. 765,255, I 20 have disclosed an apparatus employing the same compression die, but substituting for the special mold shown in said patent an ordinary one-piece mold adapted to receive a pour at a point more or less remote from 25 the compression die, with means for bodily shifting the mold and contained ingot to a position directly above the die for the lowering of the partially cooled ingot from the former into the latter.

30 In carrying out my present invention I preferably employ a compression die of the same character as that disclosed in my aforementioned patent and co-pending application; but I also employ a portable mold-support, 40 such as a car, on which an ordinary one-piece mold may receive a pour of metal at a point more or less remote from the compression die, which car and mold may be transferred to a position directly beneath the 45 die, and means located beneath the track-way of the car and in substantial axial alinement with the die whereby the partially cooled ingot may be bodily raised out of the mold and into the die for compression; thereby adopting the broad mode of 50 operation disclosed in my patent aforesaid to use in mills where the ingots are cast on a car in a casting pit.

My present invention is excellently adapted to the carrying out of a novel and useful

operation in processes of manufacture wherein the metal is first poured and partially cooled in a mold, and then transferred from the mold to a compression die to receive lateral compression.

60

Where a tapered mold is used in carrying out my present invention it is positioned on the car or other mold-support with its wide end up; and by employing a compression die with parallel walls, the greatest compression is received at the upper or wide end of the ingot, so that the resulting compressed ingot has approximately parallel, instead of tapering, sides. This effects a decided advantage in eliminating the defect known 70 as "piping," by reason of squeezing in the top end of the ingot under a pressure which is graduated from top to bottom of the ingot corresponding in a general way with the location of the pipe.

75

In the accompanying drawings I have illustrated one practical form of apparatus in and by which the invention may be practised, and referring thereto Figure 1 is a side elevation of the apparatus, in cross-section through the ingot car track and underlying pit containing the power cylinder and ram for forcing the ingot out of the mold and into the die; showing a car and ingot-mold locked thereon movable to a position directly beneath the die. Fig. 2 is a similar view, showing the ingot partially raised from the mold into the die. Fig. 3 is a top plan view of the parts shown in Fig. 1. Fig. 4 is a top plan view of the parts shown in Fig. 2.

80

Fig. 5 is a top plan view of the parts shown in Fig. 2. Referring to the drawings, I will first briefly describe the ingot press, which is a substantial duplicate of that shown in my Patent No. 1,056,101, equipped with a single 95 pair of die blocks, in lieu of the two shown in said patent.

5 designates each of a pair of parallel side frame members of the press, 6 an interlocking end frame member, and 7 a cylinder 106 casting constituting the other end frame member and formed with a pair of cylinder chambers 8 therein. The frame sections are strongly and rigidly united by interlocking joints 9 and 10 between the side and end members and by tie-rods 11. Slidably fitted within the cylinder chambers 8 are rams or plungers 12, the outer faces of which abut against a cross-head 13 that is supported on and between the side members 5 of the press 110

frame by means of flanges 14 on the cross-head resting on the upper edges of said frame members 5. The other face of the cross-head 13 in turn abuts against the back 5 of the movable die-block 15 that cooperates with a stationary die-block 16; both of said die-blocks being supported on and between the side members 5 of the press-frame by lateral flanges 17 and 18, respectively. The 10 die-blocks 15 and 16 have formed in their opposite faces V-shaped recesses 19 and 20, respectively, that unitedly form the substantial rectangular cavity of the die; the walls of the latter, as herein shown, being thus all 15 parallel with the axis of the die and vertical throughout. The die-member 15 is loosely connected to the cross-head 13 so as to be retracted by the latter by a pair of links 21.

Fluid pressure is supplied to and exhausted from the cylinder chambers 8 through a 20 cored duct 22 in the casting 7 and the pipe 23 leading from a valve 24 through which latter the pipe 23 is alternately connected with a pressure supply pipe 25 and an exhaust pipe 26. The cross-head 13 is retracted by a power mechanism comprising a cylinder 27 secured to the outer face of the inner wall casting 7, a plunger 28 in said cylinder, a cross-head 29 on the outer end of 25 said plunger, and pull-bars 30 that are connected at their outer ends to the ends of said cross-head and at their inner ends formed with hooks 31 engaging grooves 32 formed in the opposite sides of the cross head 13. A 30 branch pressure fluid supply pipe 33 leads from the supply pipe 25 to the inner end of cylinder 27, whereby the cross-head 13 is normally maintained fully retracted and the compressing die open; the cross-section of 35 the plunger 28 being so small relatively to the cross-sections of the rams 12 as to make it practically inexpedient to equip the cylinder 27 with fluid pressure controlling valves.

The compression die formed and equipped 40 substantially as above described, is mounted on any suitable substructure or support (not shown) a suitable distance above a pit 34 that may connect with or form an extension of the ordinary casting pit. Straddling the 45 pit 34 is a railway track 35, on which is adapted to travel a portable mold-support herein shown as the ordinary ingot-car 36. This car is, however, preferably modified to the extent of including lugs or stop-pieces 37 50 which serve to properly center thereon a tapered mold 38, and links 39 pivotally mounted thereon and adapted to engage at their upper ends lateral lugs 40 on the mold to hold the latter down under the stripping 55 action hereinafter described. The bottom of the mold 38 has a tapered opening 41 adapted to be closed by a tapered plug 42; and in line with the opening 41 is an opening 43 through the platform of the car to accommodate the lifting ram hereinafter described.

Within the pit 34 and in substantial axial alignment with the compression die is rigidly secured a power cylinder 44 containing the piston or head 45 of the ram 46. The cylinder 44 connects at its upper and lower 70 ends with fluid pressure pipes 47 and 48, respectively; each of which serves alternately to supply and exhaust fluid pressure to and from the cylinder from supply and exhaust pipes 49 and 50, respectively, through a controlling valve 51; this latter being capable of being turned to an intermediate position in which all of the pipes 47, 48, 49 and 50 are blanked, so as to confine a body of liquid in the cylinder 44 and hold the ram elevated 75 80 until the two members of the die have secured a good hold upon the ingot.

In preferred practice several presses would be arranged side by side with a unit spacing from center to center of the different 85 presses, and ingot cars of the general type shown would be provided of such proportions that, when coupled up in a train, their unit spacing would coincide with that of the presses, so that when a string of cars carrying one or more molds each are moved in any 90 form of tractor under the presses, the center lines of the molds and the center lines of the compressing dies are in approximate axial alignment.

In practising the invention, the cars carrying the molds are moved to the casting pit and the molds filled in the usual manner by any form of ladle which happens to be in use. After pouring is completed, the cars are moved beneath the presses and arrested at points so that the ingot-molds are directly beneath the dies. The valve 51 controlling the pit-cylinder is then turned to the position shown in Fig. 2, causing the ram 46 to ascend into contact with the plug 42 and by its further ascent to push the partly cooled ingot out of the mold and up into the compressing die, the mold itself being restrained from ascending with the ingot by the holding links 39. The controlling valve 51 is held open only long enough to permit the ingot to ascend to the proper position in the compressing die, whereupon it is then turned to blank position, thus holding the ram in its 100 elevated position. The compressing die is now brought into action to effect the lateral compression of the partly cooled ingot in the manner described in my aforesaid patent. 105 As soon as the die has obtained a good firm grip on the ingot so that it cannot drop through into the pit, the car, of course, may be drawn away, leaving the pit free.

After compression is finished the ingot may be removed from the die by either of two approved methods, one of which would consist in again applying pressure to the pit cylinder so as to bring the ram into contact with the ingot. The valve 24 would then be turned to connect the cylinders 8 with the 110 115 120 125 130

discharge pipe 26, allowing the retracting cylinder 27 to open the die, leaving the ingot loose in the latter. Pressure would then again be applied to the pit cylinder and the 5 ingot at once raised therefrom out of the die to enable the soaking-pit tongs carried by a soaking-pit crane to grasp the top of the ingot and carry it either to the soaking-pit or to a stock pile, as desired. The other method 10 of taking care of the compressed ingot would be to run an ingot car under the press and then allow the ingot to drop through the die onto this car by gravity only, the car then removing the ingot to any desired 15 place of disposal.

The die members may, of course, be made tapered to conform with the shape of the ingot; but they are preferably made with parallel side walls so that the lateral pressure 20 is applied, in a direction at right angles to the axis of the ingot and, as above stated, the compression effect extends from a maximum at the wide end of the ingot in a graduated degree to a minimum at or near the 25 narrow end of the ingot. This effects a desirable distribution and condensing of the fluid interior of the ingot that considerably facilitates the avoidance of the "piping" defect.

30 The apparatus herein described is not claimed herein, but forms the subject-matter

of a divisional application filed by me on the 21st day of November, 1913, Serial No. 802,194.

I claim—

1. A method of manufacturing ingots which consists in first casting a tapered ingot with its wide end up, and then applying lateral pressure to the partially cooled ingot in a direction at right-angles to its axis 40 while the interior of the ingot is still in a molten condition.

2. A method of manufacturing ingots which consists in first casting a tapered ingot with its wide end up, removing the ingot from the mold while in a partially cooled condition, and then subjecting the ingot to lateral pressure in a die having parallel walls while the interior of the ingot 45 is still in a molten condition.

3. A method of manufacturing ingots which consists in first casting a tapered ingot with its wide end up, removing the ingot and its mold to a position directly beneath a compression die, forcing the partially 50 cooled ingot upwardly out of the mold and into the die, and then applying lateral pressure to the ingot by means of the die.

LESLIE E. HOWARD.

Witnesses:

J. G. TABER,  
W. R. MARVIN.